

April 21, 1936.

S. L. INGERSOLL

2,038,363

IRONING SHOE AND METHOD OF MANUFACTURE THEREOF

Filed March 22, 1935

FIG. 1.



FIG. 2.



Inventor:  
Stephen L. Ingersoll,  
By *Edward R. Giffen, Jr.*

## UNITED STATES PATENT OFFICE

2,038,363

## IRONING-SHOE AND METHOD OF MANUFACTURE THEREOF

Stephen L. Ingersoll, Chicago, Ill., assignor to Borg-Warner Corporation, Chicago, Ill., a corporation of Illinois

Application March 22, 1935, Serial No. 12,385

6 Claims. (Cl. 29—148)

This invention relates to smoothing and ironing devices, and has to do more particularly with an improved laminated ironing-shoe and a method of its fabrication from different metals by a process of welding.

As presently made, ironing-shoes have a main body of relatively good heat conductive metal such as soft steel. This body is shaped as desired. One face thereof is coated with a hard 10 corrosion resistive metal to effect a smoothing surface. Usually the added metal coating or layer is chromium, and is applied by an electroplating process.

Because of the cost of applying metal coatings 15 by process of electroplating, a heavy layer is commercially impracticable; generally, it has a thickness of one or two thousandths of an inch. Such a layer can have but little resistance to lateral deformation, and, inasmuch as the only 20 reinforcement therefor is that afforded by the main body of soft steel, buttons and/or other hard objects of clothing and the like passed over the smoothing surface soon cause the plated layer to become deeply scratched, scored, and frequently punctured, rendering the shoe unfit for use. The destructive effect of hard objects of 25 this kind upon the smoothing surface of an ironing-shoe is readily conceivable when consideration is taken of the amount of force required to 30 separate the ironing-shoe and roller of an ordinary ironing machine during operation.

Partial avoidance of the difficulties experienced 35 with the use of the chromium plated shoe has been obtained by using a shoe made entirely of stainless steel. Stainless steel, however, has only approximately one-half the heat conductivity of the soft steel employed in the chromium plated shoe, so that the article formed solely of stainless steel is slow and inefficient in its transfer of heat 40 from the back to the smoothing surface thereof. When a stainless steel shoe or plate is used, more time is required to place an ironing machine in operative order. Moreover, the cost of material 45 in an ironing-shoe made entirely of stainless steel makes its use commercially prohibitive.

The primary object of the present invention is the provision of an economically produced ironing-shoe combining the wearing quality of a shoe made entirely of stainless steel, and the quality 50 of efficient heat transfer approaching that of the ordinary chromium plated shoe.

Another object of the present invention is the provision of a novel ironing-shoe clad with a non-corrosive metal readily applicable to the main 55 body of the shoe in a thickness adequate to with-

stand wear and pressure at concentrated points without becoming scratched, indented or punctured.

Another object of the present invention is the provision of a new method of producing an improved ironing-shoe as the above at a cost competitive with that of the ordinary ironing-shoe.

With the above and other desirable objects in view, the following description of a form of the invention is set forth in conjunction with the accompanying single sheet of drawing hereby made a part of this specification, and wherein:

Figure 1 is a perspective view taken angularly of an ironing-shoe constructed in accordance with the present invention; and

Figure 2 is a sectional view taken at the line 2—2 of Figure 1.

Like characters of reference are used for designating similar parts shown in the drawing and described hereinafter.

The ironing-shoe or plate 10 shown in Figures 1 and 2 of the drawing, corresponds generally in type to those commonly used in power ironing machinery. As becomes apparent upon an examination of Figure 2, the shoe 10 is substantially arcuate in transverse section, there being rolled flanges coextensive with the longitudinal edges to lessen the likelihood of the work accidentally catching upon the shoe and thereby becoming torn or injured, and to permit of the work being presented to the shoe with greater facility.

The shoe 10 is of metal and includes a main body portion 11 clad with a lamination 12 upon which is provided a smoothing surface 13. Usually the main body section 11 of the laminated shoe 10 is of soft steel, whereas the thinner section 12 is of a stainless cutlery steel suitably hardened. The section 12 may be hardened by heat treatment. Soft steel is particularly adapted as a material from which to form the main body of the shoe because of the relatively good heat conductive properties thereof. Furthermore, soft steel and stainless steel may be easily bonded together by welding or by a hot rolling process. The sections 11 and 12 of the laminated shoe may be fabricated by either of the methods described in Patents Nos. 1,868,749 and 1,967,754, issued to me July 26, 1932 and July 24, 1934, respectively, if desired.

When an ironing-shoe such as the shoe 10 is in use, heat is applied to the back side 14 thereof as by means of electrical heating units (not shown). Stub bolts 15 may be anchored to the back side of the shoe as means for securing

thereto such heating units and a protective cover (not shown) therefor. A present day ironing machine of which the illustrated ironing-shoe 10 may form a part will also include a cylindrical presser or platen member (not shown) rotatively mounted coaxially of the cylindrical portion of the shoe. Articles, such as clothing, which are to be ironed by the machine, are fed thereinto between the rotating cylindrical presser member and the smoothing surface of the shoe. Frictional engagement between the cylindrical member and the articles causes the latter to be carried by the member against and over the smoothing surface 13 of the ironing-shoe while such surface, which has been itself smoothed and polished, smoothes the articles. The smooth surface 13 of the shoe 10 effects a like surface upon the article treated thereby, and hence the shoe may be appropriately referred to as a forming-plate, and the smooth surface as a forming-surface.

Inasmuch as the two laminations 11 and 12 of the ironing-shoe 10 are interfabricated by a heating process, in contradistinction to a process of electroplating, the relative thickness of the two laminations is no factor determinative of production cost of the shoe, except with respect to the relative worth of the metals. The main body section 11 gives the shoe strength, and because of its comparative thickness, is made of a metal having a high degree of heat conductivity. In order that the obverse face of the shoe will remain smooth and unpitted from either wear or corrosion, the metal from which it is made must possess characteristics of hardness and corrosion resistivity. Steel containing chromium and sometimes a small percentage of nickel, i. e., a variety of the so-called stainless steels, has been found when properly treated for hardness, to possess the qualities required of a material for forming the obverse clad section 12 of the shoe.

The greater portion of the ironing-shoe is made of soft steel because of its low cost, its ease of combining with the stainless steel section, and its relatively good conductivity of heat. Section 12 of the shoe is made no thicker than is necessary to withstand the stress placed thereon during use. Unless the section 12 is of a certain thickness, whether it be of stainless steel or an electroplated layer, the concentrated pressure of buttons, hooks, fasteners, and the like of clothing, will cause small areas of the section to give way coincidental with being pressed into the softer counterpart body 11 of soft steel. If such were the case, deep scores and scratches would be formed in the shoe; the rustable soft iron would be exposed; and, as a consequence, the shoe's utility would be tremendously impaired. The section 12 of stainless cutlery steel, which has been hardened, is without adding appreciably to the manufacturing cost, made of a thickness to prevent its breaking down in the manner described above, and thus provides a superior form of ironing-shoe.

A particular embodiment and illustration of

the invention has been described. It is apparent, however, that other metals having similar characteristics may be joined together by a heat treating process without departing from the spirit of the invention, and so it is intended that the scope of the invention shall be limited only as defined within the appended claims.

I claim as my invention:

1. A laminated ironing-shoe having a smoothing surface provided by one of the laminations 10 thereof, said lamination being of relatively hard stainless steel, another of the laminations being of a relatively good heat conductive steel, and said laminations being fabricated to one another by a welding process. 15

2. An ironing-shoe comprising a main body section of soft heat conductive metal, and a clad section of hard corrosion-resistive metal joined to the main body section by a welding process, the clad section being shaped to provide the smoothing surface of said shoe. 20

3. The herein described process of making an ironing-shoe and comprising the steps of fabricating by welding together a relatively thick metal body having high heat conductive property 25 and a relatively thin body of hard corrosion-resistive metal, polishing the exposed surface of the corrosion-resistive metal to provide a smoothing surface, and shaping the parts thus fabricated so that the prepared smoothing surface will 30 have a section conforming to the cylindrical surface of a compressor roll.

4. The herein described process of making an ironing-shoe and comprising the steps of fabricating by welding together a relatively thick 35 metal body having high heat conductivity and a relatively thin body of hard corrosion-resistive metal, shaping the parts thus fabricated so that the corrosion-resistive metal will have an exposed surface section conforming to the cylindrical 40 surface of a compressor roll, and then polishing such exposed surface section.

5. An ironing-shoe comprising a main body section of soft heat conductive metal, and a clad section of hard corrosion-resistive metal joined 45 to the main body section by a welding process, the clad section being shaped to provide the smoothing surface of the shoe, and there being a rolled flange upon said shoe, said flange carrying a continuation of such smoothing surface. 50

6. A laminated ironing-shoe having a curved flange and having a smoothing surface provided by one of said laminations, said smoothing surface being extended onto such flange, said lamination being of relatively hard stainless steel, another of the laminations being of a relatively soft good heat conductive steel and fabricated to said stainless steel lamination by a welding process to provide a backing plate therefor, and said stainless steel lamination being of a hardness and thickness adequate to prevent indenture 55 thereof into the body of said softer lamination incident to concentrated pressure application upon limited areas thereof during use. 60

STEPHEN L. INGERSOLL. 65